

Patented Mar. 12, 1935

1,994,276

# UNITED STATES PATENT OFFICE

1,994,276

## BIMETALLIC ARTICLE

Herbert W. Graham and Samuel L. Case, Pittsburgh, Pa., assignors to Jones & Laughlin Steel Corporation, Pittsburgh, Pa., a corporation of Pennsylvania

No Drawing. Application March 16, 1933,  
Serial No. 661,092

2 Claims. (Cl. 29—181)

This invention relates to bimetallic bodies and particularly to ferrous bodies having a protective coating of tin.

Commercial tin plate is used in increasingly large amounts for containers to hold food and other commodities. As is well known, it consists of a sheet of steel which has been fed through a tin pot so as to coat both surfaces with tin. The tin represents only a very small percentage 10 of the total weight of the sheet, but if properly applied it affords substantial protection to the base metal. Tin plate as ordinarily made is open to definite limitations. For example, certain food products such as black cherries cannot be 15 successfully put up in tin cans because after a very short storage the contents of the can are discolored and the taste is spoiled, by reason of the iron in the base metal being attacked and going into solution. A great deal of difficulty 20 is also experienced in canning corn. These limitations have necessitated the use of glass containers for certain products and it has also been proposed in the case of army rations, which 25 may be shelved for a period of years before using, that stainless steel containers be employed. This, of course, is highly expensive.

Study of the problem shows that if, as is frequently the case, a very slight pin hole is present in the tin, or if the coating is thin at some point 30 and deteriorates sufficiently to allow access of moisture to the ferrous base, local electrolysis results. The action is particularly rapid if the liquid is markedly acid. Because of the relative position in the electromotive series of metals the 35 iron, rather than the tin, is attacked, discolors the contents of the can, and spoils the taste of the contents.

We have found that the difficulty can be overcome by the addition of small amounts of sodium 40 to the tin. While, as stated, the tin in ordinary

tin plate causes the iron to be attacked, we have made the surprising discovery that if sodium even in amounts as low as 0.2% is alloyed with the tin the alloy acts to inhibit the attack on the iron. Up to 2% sodium may be used. If 5 iron and tin are placed in any liquid which acts as an electrolyte, the iron will be attacked. If, however, a small percentage of sodium is added to the tin, the tin-sodium alloy saves the iron from attack. Neither tin nor sodium poisons or 10 discolors the contents of the can, or spoils its taste.

Our improved bimetallic body and containers made therefrom therefore offer numerous advantages over the ordinary tin plate or tin cans 15 of commerce, and our containers, particularly food containers, may be used for purposes where the ordinary tin can cannot be used. The shelf life of canned products is lengthened and the danger of spoilage is materially reduced. We al- 20 so believe that the presence of the sodium in the tin improves the tinning operation, resulting in a smaller percentage of waste sheets, a de- creased number of pin holes, etc.

We have described a present preferred embodiment of our invention. It will be understood, however, that this is by way of illustration only and that it may be otherwise embodied or practiced within the scope of the following claims.

We claim:

1. As a new manufacture, a food container made of a bimetallic body comprising a ferrous base and coated with a binary tin-sodium alloy, the sodium being in amount up to 2%.

2. A bimetallic body comprising a ferrous base 35 having directly applied thereto a binary alloy of tin and sodium, the sodium being present in the alloy in an amount up to 2%.

HERBERT W. GRAHAM.

SAMUEL L. CASE.

30

35

40